

C. MARK.

METHOD OF APPLYING PROTECTIVE COATINGS TO METALLIC ARTICLES.  
APPLICATION FILED JULY 29, 1915.

1,184,194.

Patented May 23, 1916.

*Fig. 1*



*Fig. 2*



Inventor

Clarence Mark

By his Attorney

Clarence Mark

# UNITED STATES PATENT OFFICE.

CLARENCE MARK, OF EVANSTON, ILLINOIS, ASSIGNOR TO CLAYTON MARK, OF CHICAGO, ILLINOIS.

## METHOD OF APPLYING PROTECTIVE COATINGS TO METALLIC ARTICLES.

1,184,194.

Specification of Letters Patent.

Patented May 23, 1916.

Application filed July 29, 1915. Serial No. 42,577.

To all whom it may concern:

Be it known that I, CLARENCE MARK, a citizen of the United States, residing at Evanston, in the county of Cook, State of Illinois, have invented a new and Improved Method of Applying Protective Coatings to Metallic Articles, of which the following is a specification, reference being had to the accompanying drawings, in which—

10 Figure 1 shows a diagrammatic representation of apparatus suitable for carrying out my improved method, and Fig. 2 is a representation of further apparatus suitable for carrying out a modification of my 15 method.

My invention relates to methods of applying protective coatings to metallic articles, such as are described and claimed in the co-pending application of Clarence Mark 20 and Clayton Mark, Jr., Serial Number 841,484, filed May 28, 1914, which has become Patent No. 1,155,317, and consists in introducing the article to be coated into a bath containing lead and zinc having superimposed thereon a layer of zinc at the point at which the article is introduced into the bath.

I have found that lead alone, or lead and tin, or lead and antimony, will not adhere 30 readily to iron or steel when low percentages of tin or antimony are used. Zinc, however, by its affinity for iron, readily unites with the iron and the resultant zinc-iron alloy forms a suitable base for adhesion of a lead-tin-zinc or lead-zinc-antimony alloy. I 35 therefore, in order to insure the formation of an adequate zinc-iron alloy on the surfaces of the article, superimpose a layer of zinc upon a portion of the alloy bath so that when the article has first been passed 40 through the zinc the alloy adheres very readily to it, and the resulting product is a very efficient one.

Referring to the drawings, in which I 45 have shown apparatus of a character suitable for carrying out my invention, A indicates a galvanizing pot or kettle, which contains a molten bath preferably composed of lead, tin and zinc, in approximately the following percentages: lead 87, zinc 3, tin 10. At one end of the receptacle A is a container B, open at top and bottom, which confines the molten zinc and separates it from the remainder of the kettle. The zinc, 55 as it is lighter than the alloy of lead, tin

and zinc, is supported and floats upon the alloy.

The articles to be treated, which I have shown in the form of pipes D, are first introduced into the zinc container B, and are pushed down through the zinc bath, and the underlying alloy bath, to the bottom of the kettle by a submerging implement C. In passing the articles through the zinc the articles will acquire enough zinc to form a zinc-iron alloy on their surfaces. They are held on the bottom until they have reached the temperature of the bath so that any unalloyed zinc will be freed therefrom, and will rise up into the container B. The submerging implement C is then tilted (as is shown in full lines in Fig. 1) to permit the articles D, because of their lighter specific gravity, to rise to the surface of the bath, outside of the container. They are then removed, and allowed to cool, and when cooled are found to have a uniform, closely adhering coating, superimposed upon the zinc-iron alloy.

In application Serial No. 841,484, which has become Patent No. 1,155,317, referred to above, a method of periodically replenishing the zinc in the bath was described and claimed. In carrying out the present process I have found that the articles will carry down sufficient zinc into the bath to keep up the desired content of zinc, so that separate additions of zinc are not required.

In Fig. 2 I have shown a type of apparatus suitable for carrying out a modification of my process, and which is particularly adapted to the treatment of articles mechanically introduced into and carried out of the bath in a rapid and continuous manner. To prevent too much zinc from being carried along through and out of the bath by the articles, I prefer to pre-heat the articles and to this end I have shown a kettle E, which may be filled with lead, or some other metal, suitable for use in pre-heating the articles. I first introduce the articles into the kettle E along a track F, so that they will be raised to approximately the temperature of the alloy bath, and I then withdraw the articles from the bath E, along the track F, and pass them through the container B', and down into and up out of the bath A'. Because of the high temperature at which the articles enter the zinc bath, a comparatively small proportion of

80

75

70

65

60

55

50

45

40

35

30

25

20

15

10

5

0

95

90

85

80

75

70

65

60

55

50

45

40

35

30

25

20

15

10

5

0

110

unalloyed zinc will adhere to the article, and so an excess of zinc will not be carried down into the alloy bath and the resulting article will accordingly not have an excess 5 of unalloyed zinc upon its surfaces.

The terms and expressions which I have employed are used as terms of description and not of limitation, and I have no intention in the use of such terms and expressions of excluding any equivalent for the 10 features shown and described, but recognize that various modifications may be made within the scope of the invention claimed.

What I claim is:

15 1. The herein described method of applying protective coatings to metallic articles, which consists of passing the article to be coated through a molten bath containing lead and zinc, the bath having super-

imposed upon it, at the point of entrance of 20 of the article, a layer of molten zinc, whereby the zinc forms with the article a zinc-iron alloy, thereby providing a base of adhesion for the alloy containing lead and zinc.

2. The herein described process of applying protective coatings to metallic articles, which consists in pre-heating the article by passing the same through a molten bath and then subsequently passing the article 30 through a second molten bath containing lead and zinc, the bath at the point of entrance of the article being covered with a layer of zinc, whereby the zinc forms a zinc-iron alloy on the article, thereby providing a base of adhesion for the alloy 35 containing lead and zinc.

CLARENCE MARK.